

## UNITED STATES PATENT OFFICE

HANS NEUMANN, OF BERLIN-SIEMENSSTADT, AND HEINRICH KÜHLEWEIN, OF BERLIN-MARIENFELDE, GERMANY, ASSIGNEES TO SIEMENS & HALSKE, AKTIENGESELLSCHAFT, OF SIEMENSSTADT, NEAR BERLIN, GERMANY, A CORPORATION OF GERMANY

## MAGNETIC ALLOY OF HIGH PERMEABILITY

No Drawing. Application filed April 25, 1931, Serial No. 532,994, and in Germany September 28, 1929.

Our invention relates to magnetic alloys of high permeability and more particularly to iron-nickel alloys.

A number of magnetic iron-nickel alloys having a high permeability for small magnetizing fields, are known. It has also already been suggested to add cobalt in quantities exceeding 4 per cent. to these alloys to increase the permeability.

10 The object of our invention is to increase the permeability still more. A further object of our invention is to obtain a particularly high constant initial permeability. Both objects are obtained by a new composition of the alloy.

The composition of the iron-nickel alloy according to the invention consists in that cobalt is added only in quantities of 0.5 to 3.5 per cent. to the iron-nickel alloys. A par-

20 ticularly great increase in the permeability is obtained according to the invention with iron-nickel alloys containing 30 to 90 per cent. of nickel, the remainder consisting of iron besides a small quantity of impurities.

25 The highest permeability is obtained with a cobalt content of about 3 per cent. and a nickel content of between 70 and 85 per cent.

With an alloy containing 76.2 per cent. of nickel, 20.9 per cent. of iron and 2.9 per cent.

30 of cobalt, for example, the following values are obtained, after the alloy has been subjected to the heat treatment hereinafter described.

35 Initial permeability 12 700  
Maximum permeability 44 200

The reversible permeability is 6 600 and the coercive force 0.06 gauss.

With an alloy containing 78.5 per cent. of nickel, 20.5 per cent. of iron and 1.0 per cent. of cobalt, the following values are obtained.

Initial permeability 7 200  
Maximum permeability 66 400

45 The reversible permeability is 7 000 to 8 000; the permeability of this alloy increases by about 10 per cent. when the field strength is increased from 0.00 to 0.01 gauss.

The heat treatment to obtain these maximum values of the permeability consists in

that the alloys are annealed at 900° C. during an hour and then slowly cooled to about 625° C., whereupon they are quenched in the air. Through this heat treatment, very high permeabilities can be reached, which are, 55 however, constant only within relatively narrow limits, as may be seen from the latter example.

By altering the heat treatment for the new alloys, it is possible to widen substantially 60 the range within which the permeability remains constant. Although the initial permeability does drop thereby to about 2 000, it is still exceedingly high, being at least five times higher than for iron. With the alloys 65 according to our invention, therefore, a high initial permeability and besides a great constancy of the permeability is obtained.

A heat treatment particularly to be recommended, is the following:

The alloy is annealed during at least an hour at a temperature of 900 to 1 100° C. and then cooled slowly during 1 to 24 hours. The slow cooling must extend to about 200° C. The further cooling may take place slowly or quickly without the properties of the alloys being substantially influenced thereby. If the last alloy mentioned above is treated in this manner the following magnetic values are obtained:

|                         |       |
|-------------------------|-------|
| Initial permeability    | 2 000 |
| Reversible permeability | 1 800 |
| Maximum permeability    | 7 800 |

Within the limits 0.00 to 0.30 gauss of the field strength, the permeability increases only 85 10 per cent. and is, therefore, practically constant in that range.

As known, the specific resistance can be increased by the addition of suitable metals, such as copper, silicon, aluminium, chromium, manganese and others. By the addition of a small quantity of silicon, the injurious influence of the carbon upon the magnetic properties may be reduced. The quantity of the said metals added to increase the specific resistance should not, however, exceed 5 per cent.

We claim as our invention:

1. A magnetic iron-nickel cobalt alloy con-

taining 0.5 to 3.5 per cent. of cobalt, 30 to 90 per cent. of nickel, the whole of the remainder consisting of iron.

2. A magnetic iron-nickel cobalt alloy containing 2.9 per cent. of cobalt, 76.2 per cent. of nickel, 20.9 per cent. of iron.

3. A magnetic iron-nickel cobalt alloy containing 1.0 per cent. of cobalt, 78.5 per cent. of nickel, 20.5 per cent. of iron.

10 4. A magnetic alloy which contains as essential ingredients iron, nickel and cobalt wherein the cobalt content is from 0.5 to 3.5%; the nickel content is from 30 to 90% and the iron content is from 6.5 to 69.5% of the entire iron-nickel-cobalt content.

15 5. A magnetic alloy, which as essential ingredients, contains iron, nickel and cobalt, the cobalt content ranging from 2.5 to 3.5%; the nickel content ranging from 70 to 85%; and the iron content ranging from 1.5 to 27.5%.

20 6. A magnetic alloy, which as essential ingredients, contains iron, nickel and cobalt and wherein the cobalt content comprises from 1 to 3.5% of the entire amount of iron, nickel, and cobalt content.

In testimony whereof we affix our signatures.

30 HANS NEUMANN.  
HEINRICH KÜHLEWEIN.

35

40

45

50

55

60